

# UNITED STATES PATENT OFFICE.

CARLETON ELLIS, OF MONTCLAIR, NEW JERSEY, ASSIGNOR TO CHADELOID CHEMICAL COMPANY, OF NEW YORK, N. Y., A CORPORATION OF WEST VIRGINIA.

## FINISH-REMOVER.

1,118,642.

Specification of Letters Patent. Patented Nov. 24, 1914.

No Drawing.

Application filed April 1, 1912. Serial No. 687,770.

To all whom it may concern:

Be it known that I, CARLETON ELLIS, a citizen of the United States, and resident of Montclair, county of Essex, and State of New Jersey, have made a certain new and useful Invention Relating to Finish-Removers, of which the following is a specification.

This invention relates especially to finish removers comprising phenol camphor or similar compounds, together with incorporated volatile organic solvent material and waxy or other suitable stiffening material if desired. Various solid camphor terpenes have the peculiar property of combining with phenols in definite proportions so as to form compounds which have distinctive properties widely different from the components used. Ordinary laurel camphor, Borneol camphor and the turpentine camphors or their derivatives may be combined in this way with carbolic or cresylic acids. For instance, pure crystallized carbolic acid which melts at 43° C. when combined with laurel camphor which melts at 175° C. forms a liquid solvent melting much below zero. Such combinations may be effected when the two components are triturated or otherwise intimately incorporated as by being brought together in solution which naturally expedites this combination. In removers, for instance, these camphorate solvents may be first formed and then incorporated with other remover ingredients or may be conveniently formed by bringing the components together in solution with the other remover ingredients. These camphoric terpenes seem to combine most readily in equimolecular proportions, although not only a camphorate but a bicamphorate can be formed with carbolic acid or with other phenols, such, for instance, as cresylic acid. These compounds are heavy liquids having a very general and desirable solvent action on many paint or varnish gums, resins or binders so as to be desirable components for finish removers. It is also desirable to incorporate a suitable small proportion of such practically non-volatile material in removers to prevent any possibility of the drying out of finish on which waxy removers have acted to soften or loosen the same.

In this way even under extreme service conditions it is practically impossible for the wax or treated finish to form an undesirably hard coating even if allowed to stand for unusually long periods.

The main remover solvents may comprise loosening finish solvent material, that is solvents of a generally alcoholic character or action in removers, such as methyl, ethyl, propyl, butyl, benzyl and other strict alcohols, preferably in their commercial forms, including denatured alcohol as well as ketonic solvents, such as methyl, ethyl, ketone, oil of acetone, acetone, methyl acetone and higher ketone finish solvents; and the corresponding esters may also be used, such as methyl acetate, ethyl acetate and chlorinated derivatives, such as chlorinated methyl acetone, which is an oily solvent body largely insoluble in water. Suitable penetrating finish solvent material may also be used, that is solvent material of a generally benzolic character or action in removers, such as benzol and its homologues, toluol, xylol and their commercial forms, such as commercial toluol, solvent naphttha and the somewhat analogous petroleum hydrocarbons, such as naphtha and benzin and the chlorinated derivatives, such as chlorbenzol, chlortoluol and other chlorinated solvents, such as carbon-tetrachlorid, tetrachlorethane and the like, and also turpentine, wood turpentine and various esters and ethers, such as betanaphthol ether, benzyl ethers, xylol ethers, phenol ethers, Borneol ethyl ether, anilin acetate, anilin phenate, or other liquid solvent anilin compounds, guaiacol and the bodies formed by deodorizing and treating wood tar oils, wood turpentine, pine oil and so forth, by nascent hydrogen as by agitation of the solvent with sodium, potassium or the like or by other treatment with hydrogen in the presence of active metallic material, such as platinum, palladium and so forth. Suitable heavy solvents, such as may be used to minimize any tendency to drying out of the remover may comprise epichlorhydrin, dichlorhydrin or chlorinated glycerole or ethyl or methyl phenates. Ethyl phenate and methyl phenate and the corresponding cresylates are also desirable solvents which may

be conveniently produced in various ways, the combination of the components being facilitated by suitable catalytic material such as aluminum oxid, thorium oxid or the like 5 at a temperature of 350° to 400° C. or so, the thorium oxid having especially desirable catalytic action in this connection and promoting the formation of these particular compounds when the components are 10 brought together in this way.

Suitable stiffening material may be used in such removers preferably comprising suitable waxy evaporation-retarding material, such as paraffin, ceresin or other mineral wax, although beeswax and other waxy bodies may be used and also other stiffening material, such as cellulose esters, including nitrocellulose, which may be used in the form of scrap celluloid which usually contains 15 nitrocellulose and sufficient incorporated camphor to combine with phenol and form the camphorated solvents referred to. Inert stiffening material may also be incorporated if desired, such for example as wood flour, starch, infusorial earth, whiting and the like, it being of course understood that the soluble thickeners are preferably first dissolved in the more energetic solvents therefor with a slight increase of temperature if desired and then the other components incorporated and energetically mixed to secure uniformity.

An illustrative composition of this character may comprise 20 parts of methyl alcohol, 25 parts of acetone, 20 parts of ethyl or methyl acetate, 20 parts of benzol, 10 parts of benzyl alcohol, 4 parts of laurel camphor, 10 parts of scrap celluloid which would contain nitrocellulose, and about 4 35 parts of camphor, 6 parts of carbolic acid and 2 parts of paraffin. Another illustrative remover may comprise 20 parts of acetone, 20 parts of methyl acetone, 30 parts of benzol, 15 parts of ordinary camphor, 10 40 parts of carbolic acid and 5 parts of paraffin. Another illustrative composition may comprise 30 parts of acetone, 25 parts of benzol, 30 parts of laurel or Borneol camphor and 20 parts of carbolic or cresylic acid and 3 to 50 5 parts of paraffin or ceresin wax. Another illustrative composition suitable for general purposes may comprise 20 parts of chlorinated methyl acetone or of tetrachlorethane, 20 parts of acetone, 35 parts of benzol, 55 2 parts of laurel camphor, 2 parts of celluloid scrap, 4 parts of carbolic acid and 2 to 3 parts of paraffin. Another generally useful composition may comprise 30 parts of methyl alcohol, 30 parts of acetone, 40 parts of benzol, 60 10 parts of celluloid scrap, 4 parts of carbolic or cresylic acid and 1 part of paraffin or ceresin wax. Another illustrative composition may comprise 40 parts of acetone, 20 parts of benzol, 30 parts of camphor, 20 parts of carbolic acid and 3 parts 65

of paraffin. Another illustrative composition may comprise 60 parts of camphor and 40 parts of carbolic or cresylic acid. Another illustrative composition may comprise 30 parts of denatured alcohol, 20 parts of carbon-tetrachlorid, 30 parts of benzyl alcohol, 20 parts of laurel camphor, 5 parts of scrap celluloid, 2 parts of paraffin and 15 parts of carbolic acid. 70

Having described this invention in connection with a number of illustrative ingredients, formulas, proportions and processes, to the details of which disclosure the invention is not of course to be limited, what is claimed as new is:

1. The finish remover comprising approximately 20 parts of methyl alcohol, 10 parts of benzyl alcohol, 25 parts of acetone, 20 parts of methyl acetate, 20 parts of benzol, 4 parts of laurel camphor, 10 parts of celluloid containing about 4 parts of camphor, 6 parts of carbolic acid and 2 parts of paraffin. 80

2. The finish remover comprising approximately 30 parts of alcohol, 25 parts of acetone, 20 parts of methyl acetate, 20 parts of benzol, 4 parts of camphor, 10 parts of celluloid scrap containing camphor, 6 parts of phenol combined with such camphor to form a liquid finish solvent compound and 95 mineral wax. 90

3. The finish remover comprising approximately 90 parts of volatile organic finish solvent material comprising an alcohol, 4 parts of camphor, 10 parts of celluloid comprising camphor, phenol combined therewith and incorporated wax. 100

4. The finish remover consisting in greater proportion of loosening finish solvent material comprising a ketone, aromatic penetrating solvent material, celluloid containing camphor, phenol combined therewith and incorporated waxy material. 105

5. The finish remover consisting in greater part of volatile finish solvent material, including ketonic finish solvent material, celluloid containing camphor, carbolic acid combined therewith and incorporated waxy material. 110

6. The finish remover consisting in greater proportion of volatile organic finish solvent material, celluloid containing pyroxylin and camphor, and phenol combined therewith. 115

7. The substantially non-aqueous finish remover comprising liquid finish solvent material, solid camphoric terpene material capable of combining with phenol and carbolic acid combined therewith. 120

8. The finish remover comprising in larger part liquid organic finish solvent material, solid camphoric terpene material capable of forming a liquid finish solvent by combination with carbolic acid and phenol combined therewith. 125

9. The finish remover consisting in greater 130

part of volatile organic finish solvent material comprising a finish solvent ketone, solid camphoric terpene material and phenol combined therewith to form a liquid finish 5 solvent compound.

10. The finish remover consisting in greater part of volatile organic finish solvent material and comprising a liquid finish solvent camphoric compound formed by combining camphor and carbolic acid.

11. The finish remover comprising a liquid finish solvent-camphoric compound formed by combining a solid camphoric terpene material with phenolic material.

15. 12. The liquid solvent suitable for use in dissolving or softening finish material comprising solid camphoric terpene material and phenolic material combined therewith.

13. The liquid solvent suitable for use in 20 dissolving or softening finish material comprising camphor and carbolic acid combined therewith.

14. The finish remover comprising volatile organic finish solvent material, pyroxylin, camphor, phenol combined therewith and incorporated wax.

25. 15. The finish remover consisting in

greater part of volatile composite finish solvent material including benzol and acetone, celluloid containing camphor, phenol 30 and incorporated wax.

16. The substantially non-aqueous finish remover consisting in greater part of volatile organic finish solvent material and comprising a liquid finish solvent camphoric 35 compound formed by combining a solid camphoric terpene material with carbolic acid.

17. The substantially non-aqueous finish remover consisting in greater part of volatile organic finish solvent material and comprising a liquid finish solvent camphoric compound formed by combining a solid camphoric terpene material with carbolic acid, 40 and incorporated wax.

18. The finish remover consisting in 45 greater proportion of volatile composite organic finish solvent material comprising acetone and a miscible aromatic solvent, celluloid containing camphor and incorporated carbolic acid and waxy material.

CARLETON ELLIS.

Witnesses:

HARRY L. DUNCAN,  
JESSIE B. KAY.